

## UNITED STATES PATENT OFFICE.

YOTARO FUJITA, OF KYOTO, JAPAN.

## MANUFACTURE OF ADHESIVE METALLIC POWDER IN THE FORM OF METALLIC SCALES.

No Drawing.

Application filed April 28, 1922. Serial No. 557,181.

*To all whom it may concern:*

Be it known that YOTARO FUJITA, a subject of the Emperor of Japan, residing at city of Kyoto, Japan, has invented certain 5 new and useful Improvements in the Manufacture of Adhesive Metallic Powder in the Form of Metallic Scales; and he does hereby declare the following to be a full, clear, and exact description of the invention, such as 10 will enable others skilled in the art to which it appertains to make and use the same.

This invention relates to the manufacture of adhesive metallic powder in the form of metallic scales to be used for applying, in 15 scattered manner, to the surface of cloth or paper in order to make any required design thereon.

To make a design with metallic powder formed of metallic scales by applying the 20 same to the surface of cloth or paper in scattered manner, heretofore the powder was either scattered in any convenient way on the surface of a cloth or paper on which an adhesive paste had been applied, or was 25 homogeneously mixed with liquid-paste and painted on the surface. But according to my invention the metallic scales forming the powder are coated on one surface with an adhesive agent which melts by heat. If the scales 30 thus coated are scattered over the surface of cloth or paper, a part of them set with the coated surface upwards and the other downwards. So that, if another sheet of cloth or paper is placed upon the surface on which 35 the scales have been scattered, and then pressed by a hot trowel passed thereover, the coating agent again melts firmly sticking the scales to the surface of the sheets. As it is easily understood, some of the scales 40 stick to the surface of the upper sheet while the others to that of the lower one, thus the same but opposite, or symmetrical, design by the scattered scales may be obtained simultaneously on the two sheets.

45 The new powder in the form of metallic scales may be manufactured as follows:

A large metallic leaf is flatly placed, either temporarily coated with paraffin or not, upon a sheet of strong paper, and fine powder of an agent, which easily melts by heat, such as 50 lac or gum, is evenly put all over the surface of the leaf. When the leaf together with the sheet of paper is heated, the powdered agent will melt and cover the whole surface of the leaf as an adhering coating. 55 Then it is cooled down, and the paper beneath the leaf is taken off.

The leaf thus obtained is coated with a film of the agent on one side, the other side being left uncovered. By grinding this leaf 60 in a well known manner into powder of a required grade, metallic scales, one side of which are equipped with a film of the adhesive agent, are finally obtained.

What I claim is:—

1. A process for preparing an adhesive metallic powder in the form of metallic scales comprising putting fine powder of an adhesive agent, which melts by heat, upon a large leaf of metal, heating the leaf so as to 70 melt the powdered agent and form a coating thereof upon the leaf, and grinding the leaf into powder of a required grade.

2. A process for preparing an adhesive powder in the form of metallic scales comprising placing a large metallic leaf on a strong paper, putting fine powder of an agent, which easily melts by heat, upon the leaf, heating the same so as to melt the powdered agent and form a coating of the agent 75 thereon, taking off the paper, and grinding the leaf into powder of a required grade.

3. As a new product, adhesive metallic scales, one surface of which is coated with a film of an adhesive agent, which melts by 80 heat.

In testimony whereof I hereunto affix my signature.

YOTARO FUJITA. [L. s.]

Witnesses:

W. EBiharah,  
TAKATUGU HIGASHINA,